# EUROPEAN PATENT SPECIFICATION

(11) **EP 2 503 038 B1**
(45) Date of publication and mention of the grant of the patent: **26.10.2022**
(21) Application number: 11169951.8
(22) Date of filing: 15.06.2011
(51) Int. Cl.: D06M 10/00, D06M 23/08, D03D 15/58, D03D 15/00, D03D 1/02

(54) **A fabric for an air-bag and method for manufacturing the fabric**
Stoff für einen Airbag und Herstellungsverfahren für den Stoff
Tissu pour airbag et procédé de fabrication du tissu

(30) Priority: 23.03.2011 EP 11159477
(43) Date of publication of application: 26.09.2012
(73) Proprietor: Autoliv Development AB, 447 83 Vårgårda (SE)
(72) Inventor: Finn, Hugh, Culcheth, Warrington, Cheshire WA3 4LG (GB); Koehnen, Ralf, Congleton, Cheshire CW12 4FJ (GB)
(74) Representative: Forresters IP LLP

(56) References cited:
- EP-A1- 0 095 537
- EP-A1- 0 442 373
- JP-A- H06 184 856
- US-A- 2 245 641
- US-A- 5 183 703
- US-A- 5 236 775

## Description

### Description of Invention

THIS INVENTION relates to a method for manufacturing an air-bag, and in particular concerns a method for weaving a fabric for use in the production of air-bags.

Currently vehicle air-bags are generally formed from woven nylon fabric. The fabric is typically manufactured by drawing a number of parallel warp yarns from a reel, and weaving weft yarns across the warp yarns, generally at right angles thereto. A first weft yarn will be woven into the warp yarn so that it passes over and under alternate warp yarns. The next weft yarn will be introduced so that it passes over the warp yarns that the first weft yarn passed under, and *vice versa.*

These fabrics are generally prepared using large, dedicated weaving looms, which will be well-understood by those skilled in the art.

The warp yarns are subject to friction and abrasion as they pass through the loom, through coming into contact with neighbouring yarns and against components of the loom. It is therefore necessary to protect the warp yarns from damage during the weaving process.

In general, this is achieved by forming each warp yarn from a relatively large number of filaments (for example, around 140 filaments). These filaments are extruded and gathered together to form the yarn, and the yarn is nipped at periodic intervals to form points of entanglement. These periodic entanglement points may be provided at a spacing of around 20 to 30 per metre of yarn.

The warp yarns then have coating applied to protect them during the weaving process. This coating is known as the "size", and is applied by passing the yarn through a size bath. Typically, the size may form around 0.5 to 2% by weight of the finished yarn.

Once the yarn has been woven into a fabric, the size is removed from the fabric during a scouring process, in which chemicals are applied to the fabric to dissolve the size and wash the size away.

US5236775 and EP0442373 disclose an airbag fabric made of a synthetic yarn. The synthetic yarn is a high-tenacity polyester filament yarn having filaments of less than 4 dtex and a yarn count within the range from 250 to 550 dtex. The fabric itself, in contrast to the conventional polyamide fabrics, is uncoated and is preferably made by weaving unsized yarns. The fabric need not be calendered. It has been found that this fabric of fine-filament high-tenacity polyester yarn, although uncoated, does meet the airbag fabric requirements such as low air permeability, low fabric weight, low fabric thickness and high fabric strength.

EP0095537 discloses a high twist polyester multifilament yarn having a twist of a twist multiplier K within a range between 15,000 and 25,000, made from polyester filaments consisting essentially of a copolymer of two or more monomers selected from the group consisting of ethylene terephthalate, trimethylene terephthalate and tetramethylene terephthalate and/or a blend of two or more polymers of the respective monomers and having a breaking elongation of not more than 60% and shrinkage in boiling water of not more than 6%. A woven or knitted crepe fabric obtained by employing such a high twist yarn has a desirable pebble configuration.

US2245641 discloses a composite yarn and a fabric made from the composite yarn. The yarn is twisted by at least 10-12 turns per inch (per 2.5 cm). US5183703 discloses belt strap for safety belts which is to have outer surfaces of as low friction as possible so that it can run through the safety belt system with as little friction as possible. The warp threads, which are woven into the belt strap, have filaments of at least 15 dtex, particularly 17 dtex. The warp threads are, in one embodiment, untwined and tangled at certain points with compressed air, whereby the tangled points can be spaced from one another by 5 to 15 cm. In another embodiment the warp threads are twined only slightly, namely with 30 to 50 twists per metre thread length.

JPH06184856 discloses a conventional low air-permeable woven fabric and its production.

It is an object of the present invention to provide an improved method for weaving a fabric for use in vehicle air-bags.

According to one aspect of the present invention, there is provided an air-bag as defined in claim 1 hereinafter.

In order that the present invention may be more readily understood, embodiments thereof will now be described, by way of example, with reference to the accompanying drawings, in which:
Figure 1 is a schematic view of a warp yarn suitable for use with the present invention; and
Figure 2 is a schematic view of a fabric embodying the present invention.

With reference firstly to figure 1, a yarn 1 is shown which is suitable for use as a warp yarn in embodiments of the present invention. The yarn 1 is formed from a number of individual filaments 2 which are twisted together to form the yarn 1. Either "S" or "Z"-twists (i.e. right-or left-handed twists) may be used to form the yarn 1.

In preferred embodiments the yarn 1 consists of a bundle of around 96 to 120 filaments 2. The number of filaments 2 in the yarn 1 may be as high as 180 or even higher, however.

Preferably, the degree of twist of the yarns 2 is between around 40 and 200 turns per metre of the yarn 1. If the degree of twist is less than around 40 turns per metre, it has been found that there is generally insufficient consolidation of the filaments 2 that make up the yarn 1.

On the other hand, if the degree of twist is greater than around 200 turns per metre, it has been found that the resulting yarn becomes too heavy, stiff and unwieldy to be woven effectively into a fabric. In addition the high level of twist will reduce the throughput of the twisting machine, thus increasing the cost.

In order to form the yarn 1, the filaments 2 forming the yarn are extruded in the normal (or any suitable) manner, and are nipped at periodic intervals to form entanglement points. The bundle of filaments is then sent to a twisting machine, which twists the filaments together to form the yarn 1. Before or after this twisting process the yarn 1 may be passed through a size bath so that a suitable finish or lubricant can be applied to the yarn 1. The finished yarn 1 is then wound on to a bobbin, which can then be used to transport the yarn 1 to its destination.

The yarn 1 is then used as warp yarns in a weaving process to form a fabric, as discussed above.

Figure 2 shows a close-up view of a region of woven fabric 3 embodying the present invention. Figure 2 is a schematic figure and the size and spacing of the yarns forming the fabric 3 is exaggerated for the purpose of clarity.

The fabric 3 is formed from a series of warp yarns 4, which run vertically in figure 2, and weft yarns 5, which run horizontally in figure 2. As will be understood by those skilled in the art, each warp yarn 4 passes alternately over and under each alternate weft yarn 5 that is encountered along the length of the warp yarn 4. Similarly, each weft yarn 5 passes alternately over and under each warp yarn 4 that is encountered along the length of the weft yarn 5.

Each warp yarn 4 is formed from a bundle of twisted filaments, as shown in figure 1. Each weft yarn 5 is substantially untwisted, comprising a bundle of filaments which are generally parallel to one another, and have a degree of twist which is less than about 5 turns per metre.

Fabrics embodying the present invention will have warp yarns that are more robust, in which the filaments forming the warp yarns hold together more readily, and are more resistant to damage through friction and abrasion during the weaving process. This means that a reduced amount of size, or no size, may be applied to the warp yarns prior to the weaving process beginning, thus reducing the cost of the finished fabric, both in the amount of size that has to be added to the warp yarns prior to weaving and also in the degree of scouring that needs to be performed to remove the size from the fabric after weaving has been completed.

It is anticipated that the present invention will be a particular application to fabrics formed from polyester. As mentioned above, conventional fabrics for vehicle air-bags are formed from nylon, and the majority of looms and other weaving equipment are configured to process yarns formed from filaments of nylon. However, nylon is relatively expensive, and it would be preferable to employ cheaper materials such as polyester.

Polyester is stiffer than nylon, and periodic entanglements cannot be applied to polyester as effectively. Periodic entanglements can generally only be applied to polyester yarns with a frequency of around 9 to 20 entanglements per metre. Also, because the filaments forming the yarn are stiffer, the entanglement points do not bind the filaments together as reliably.

In addition, the size that is used for coating nylon yarns can generally not be applied directly to polyester yarns. The size required to coat polyester yarns is more expensive, and present scouring machines are not configured to remove this size effectively. It is therefore desirable to use as little size as possible, or no size, and as discussed above a reduction in the required amount of size can be achieved by forming the warp yarns from twisted filaments.

In embodiments of the invention the weft yarns are substantially untwisted. This is because the weft yarns are, in general, not subject to friction and/or abrasion to the same degree as warp yarns during the weaving process, and are not as prone to breakage of filaments. The twisting stage, which inevitably increases the cost of yarn, need therefore not be applied to the weft yarns.

In addition, in preferred embodiments the weft yarns do not have any size applied thereto. However, the weft yarns may have a relatively small amount of finish or lubricant, for instance around 0.5% of "spin finish" from the manufacturing stage.

In preferred embodiments, one or both of the warp and weft yarns are formed to have a density of around 400 to 600 decitex. However, the decitex may be considerably higher, for instance up to around 1800 decitex, or may be lower, for instance around 167 decitex.

It is anticipated that fabrics embodying the present invention will find utility in various forms of vehicle air-bag, including (but not limited to) internal passenger protection air-bags and external pedestrian protection air-bags. Embodiments of the invention provide air-bag modules including air-bags formed entirely or partially from fabrics as described above.

## Claims

1. An air-bag formed from a fabric (3) which is formed from interwoven warp and weft yarns (1, 4; 5) which are arranged to be substantially perpendicular to one another, wherein the warp yarns (1, 4) are formed from multiple filaments which are twisted together to form the warp yarns (1, 4), with a degree of twist of about 40 turns per metre, **characterised in that** the weft yarns (5) are
substantially untwisted, and wherein the degree of twist of the weft yarns (5) is less than about 5 turns per metre.

2. An air-bag according to claim 1, wherein every successive warp yarn (1, 4) is formed from filaments that are twisted together.

3. An air-bag according to claim 1 or claim 2, wherein the warp yarns (1, 4) have periodic entanglement points, at which the filaments forming the yarns (1, 4) are entangled together.

4. An air-bag according to claim 3, wherein fewer than about 20 entanglement points per metre of warp yarn (1, 4) are formed.

5. A method of forming an air-bag, comprising:
forming warp yarns (1, 4) by:
providing a bundle of filaments (2);
gathering the bundle of filaments (2) together; and
twisting the filaments (2) together, by a degree of twist of around 40 turns per metre, to form the yarn (1, 4);
providing a plurality of weft yarns (5) which are substantially untwisted, wherein the degree of twist of the weft yarns (5) is less than about 5 turns per metre;
weaving the warp and weft yarns (1, 4; 5) together to form a fabric (3), so that the warp and weft yarns (1, 4; 5) are arranged to be substantially perpendicular to one another; and
forming an air-bag from the fabric (3).

6. A method according to claim 5, further comprising the step of applying periodic entanglement points to the bundle of filaments (2), prior to the twisting step, the filaments (2) being entangled with one another at the entanglement points.

7. An air-bag module comprising an air-bag according to any one of claims 1 to 4.

8. A vehicle comprising an air-bag module according to claim 7.

## Patentansprüche

1. Airbag, der aus einem Stoff (3) ausgebildet ist, der aus durchwobenen Kett- und Schussgarnen (1, 4; 5) ausgebildet ist, die angeordnet sind, um im Wesentlichen senkrecht zueinander zu sein, wobei die Kettgarne (1, 4) aus mehreren Filamenten ausgebildet sind, die miteinander verdreht sind, um die Kettgarne (1, 4) mit einem Verdrehungsgrad von etwa 40 Verdrehungen pro Meter auszubilden, **dadurch gekennzeichnet, dass** die Schussgarne (5) im Wesentlichen nicht verdreht sind und wobei der Verdrehungsgrad der Schussgarne (5) weniger als etwa 5 Verdrehungen pro Meter beträgt.

2. Airbag nach Anspruch 1, wobei jedes aufeinanderfolgende Kettgarn (1, 4) aus Filamenten ausgebildet ist, die miteinander verdreht sind.

3. Airbag nach Anspruch 1 oder 2, wobei die Kettgarne (1, 4) periodische Verwicklungspunkte aufweisen, an denen die Filamente, die die Garne (1, 4) ausbilden, miteinander verwickelt sind.

4. Airbag nach Anspruch 3, wobei weniger als etwa 20 Verwicklungspunkte pro Meter Kettgarn (1, 4) ausgebildet sind.

5. Verfahren zum Ausbilden eines Airbags, umfassend:
Ausbilden von Kettgarnen (1, 4) durch:
Bereitstellen eines Bündels von Filamenten (2);
Zusammensammeln des Bündels von Filamenten (2); und
Zusammenverdrehen der Filamente (2) mit einem Verdrehungsgrad von etwa 40 Verdrehungen pro Meter, um das Garn (1, 4) auszubilden;
Bereitstellen einer Vielzahl von Schussgarnen (5), die im Wesentlichen nicht verdreht sind, wobei der Verdrehungsgrad der Schussgarne (5) weniger als etwa 5 Verdrehungen pro Minute beträgt;
Zusammenweben der Kett- und Schussgarne (1, 4; 5), um einen Stoff (3) auszubilden, sodass die Kett- und Schussgarne (1, 4; 5) angeordnet sind, um im Wesentlichen senkrecht zueinander zu sein; und
Ausbilden eines Airbags aus dem Stoff (3).

6. Verfahren nach Anspruch 5, ferner umfassend den Schritt eines Aufbringens periodischer Verwicklungspunkte auf das Bündel von Filamenten (2) vor dem Verdrehungsschritt, wobei die Filamente (2) an den Verwicklungspunkten miteinander verwickelt sind.

7. Airbagmodul, umfassend einen Airbag nach einem der Ansprüche 1 bis 4.

8. Fahrzeug, umfassend ein Airbagmodul nach Anspruch 7.

## Revendications

1. Coussin gonflable de sécurité formé à partir d'un tissu (3) qui est formé à partir de fils de chaîne et de trame entrelacés (1, 4 ; 5) qui sont agencés pour être sensiblement perpendiculaires les uns aux autres, dans lequel les fils de chaîne (1, 4) sont formés à partir de multiples filaments qui sont torsadés ensemble pour former les fils de chaîne (1, 4), avec un degré de torsion d'environ 40 tours par mètre, **caractérisé en ce que** les fils de trame (5) sont sensiblement non torsadés, et dans lequel le degré de torsion des fils de trame (5) est inférieur à environ 5 tours par mètre.

2. Coussin gonflable de sécurité selon la revendication 1, dans lequel chaque fil de chaîne successif (1, 4) est formé à partir de filaments qui sont torsadés ensemble.

3. Coussin gonflable de sécurité selon la revendication 1 ou la revendication 2, dans lequel les fils de chaîne (1, 4) ont des points d'enchevêtrement périodiques, au niveau desquels les filaments formant les fils (1, 4) sont enchevêtrés ensemble.

4. Coussin gonflable de sécurité selon la revendication 3, dans lequel moins d'environ 20 points d'enchevêtrement par mètre de fil de chaîne (1, 4) sont formés.

5. Procédé de formation d'un coussin gonflable de sécurité, comprenant :
la formation de fils de chaîne (1, 4) par :
la fourniture d'un faisceau de filaments (2) ;
le rassemblement du faisceau de filaments (2) ; et
la torsion des filaments (2) ensemble, selon un degré de torsion d'environ 40 tours par mètre, pour former le fil (1, 4) ;
la fourniture d'une pluralité de fils de trame (5) qui sont sensiblement non torsadés, dans lequel le degré de torsion des fils de trame (5) est inférieur à environ 5 tours par mètre ;
le tissage des fils de chaîne et de trame (1, 4 ; 5) ensemble pour former un tissu (3), de sorte que les fils de chaîne et de trame (1, 4 ; 5) sont agencés pour être sensiblement perpendiculaires les uns aux autres ; et
la formation d'un coussin gonflable de sécurité à partir du tissu (3).

6. Procédé selon la revendication 5, comprenant en outre l'étape d'application de points d'enchevêtrement périodiques au faisceau de filaments (2), avant l'étape de torsion, les filaments (2) étant enchevêtrés les uns avec les autres au niveau des points d'enchevêtrement.

7. Module de coussin gonflable de sécurité comprenant un coussin gonflable de sécurité selon l'une quelconque des revendications 1 à 4.

8. Véhicule comprenant un module de coussin gonflable de sécurité selon la revendication 7
